

March 23, 1965

R. P. CULBERTSON

3,175,074

ELECTRIC ARC WELDING

Filed Oct. 3, 1962



Fig. 1.



Fig. 2.



Fig. 3.

INVENTOR.  
RUSSEL P. CULBERTSON

BY *Barnwell P. King*

ATTORNEY

## 1

3,175,074

**ELECTRIC ARC WELDING**

Russel P. Culbertson, Kokomo, Ind., assignor to Union Carbide Corporation, a corporation of New York  
 Filed Oct. 3, 1962, Ser. No. 228,637  
 8 Claims. (Cl. 219—146)

This invention relates to work-in-circuit electric arc welding, and more particularly to the art of hard-facing articles subjected to severe wear, such as railroad rails.

The invention provides a cored-wire electrode for semi-automatic electric arc welding, especially building up worn rail ends in situ, without the need for any shielding gas stream, in which the core-material is a powder-blend of —30 screen size metal powder and free carbon in an amorphous state, the particles of which approach the molecular by virtue of the grinding which takes place with the metal powder in the mixing-blending process which also uniformly distributes and disburses such carbon throughout the core. As a result, the welding operation is simpler, cheaper, and may be done by even inexperienced welders. Furthermore, the weldments are superior in that they withstand battering in severe railroad service for a much longer time than was possible according to the prior art even in the cases of  $\text{CO}_2$  and argon stream arc shielding.

In industry, the replacement and maintenance of components due to wear of metal parts is a formidable and costly problem. The railroad industry must constantly service or replace rails because of wear. Only a slight amount of wear is caused by the wheels rolling over the rails. At the rail ends, however, wear is excessive because of the batter of the wheels as they pass over the rail joint and drop on the succeeding rail. As wear increases, the batter becomes more severe, thereby accelerating more wear in a vicious circle.

The constant batter of the wheels on the rail ends causes loosening of rail ties, an uneven ride of the railroad cars and promotes the formation and growth of transverse fissures, detail fractures and gauge corner shelling of the rails, which often result in rail failure in service. Such types of rail damage usually originate as small internal imperfections in the rail that produce minute cracks, these cracks grow larger by a fatigue failure mechanism caused by stresses, vibrations and batter, especially at the rail ends.

Several means are available to reduce rail failures described above. (1) Reduction of the number of rail joints by increasing rail lengths from 33 feet to 39 feet or more. (2) Rail joints may be also reduced by the formation of continuous rail by joining rail ends by thermit welding and resistance butt welding, which are costly and cumbersome to perform at the scene of installation. (3) Rail failures may be reduced by heating, quenching and tempering the entire rail or at least the rail ends. However, because rails are produced by hot rolling into final shape in lengths of over 33 feet, such heat-treatment would be costly and difficult and may result in warpage of the rail. (4) The most practical available means of reducing the above-mentioned rail failures appears to be in fusion coating the worn areas of the rail ends with an alloy that is resistant to wear and compatible with the composition of the original rail as shown in Table I.

## 2

TABLE I

 Composition and hardness of typical rails<sup>1</sup>

[U.S. Standard Rails]

|                 | Composition in Weight Percent |         |         |
|-----------------|-------------------------------|---------|---------|
|                 | Maximum                       | Minimum | Average |
| Carbon.....     | 0.88                          | 0.70    | 0.80    |
| Manganese.....  | 0.98                          | 0.72    | 0.85    |
| Silicon.....    | 0.30                          | 0.11    | 0.17    |
| Phosphorus..... | 0.038                         | 0.008   | 0.016   |
| Iron.....       | Bal.                          | Bal.    | Bal.    |
|                 | Hardness, Brinell             |         |         |
|                 | 302                           | 225     | 257     |

<sup>1</sup> Compiled data representing about 70 heats of standard rails from eight railroads.

20 This invention provides novel filled tube rod or wire electrodes, preferably in the form of coils which are applied by the open-arc process. The electrode is preferably made according to the method of Stoody Patent No. 1,629,748, dated May 24, 1927. One of the outstanding advantages of the open-arc process is the elimination of any need for an inert gas supply and attendant equipment. This feature is especially desirable for welding and hard-surfacing operations that are performed away from the shops, for example, field maintenance of railway track members. In the open-arc process there is no gas shielding; therefore, the tube electrode filler usually contains an organic powder (wood or other vegetable products) or an inorganic powder such as siderite ( $\text{FeCo}_3$ ) or limestone (calcium carbonate). Such powders are consumed and/or sublimated by the heat of the arc, thereby providing an effective gaseous envelope (primarily CO and  $\text{CO}_2$ ) to protect the arc stream and the deposit puddle.

25 The use of the general class of organic and inorganic powders mentioned above has limitations that prevent a broader exploitation of the open-arc process, which is more efficient and more economical than other comparable welding methods.

30 Tube electrodes that contain the above-mentioned organic and inorganic filler materials, which provide a protective gaseous envelope in open-arc processes, are used for many applications in industry. However, deposits made from prior materials often vary widely in composition and physical and mechanical properties. Because of such prior limitations, the railroad industry has preferred that right-of-way rail welding and surfacing be performed by inert-gas-shielded methods. Such methods assure more uniform deposits of the highest degree of quality and dependability, thus minimizing rail failures. Thus, there is a great need for a tube rod that meets the stringent requirements of the railroad industry and may be applied by the open-arc process more efficiently and more economically.

35 The primary object of this invention is to provide an improved composition for filler tube rods or coils.

40 Another important object is to provide a welding or surfacing electrode suitable for application on railway right-of-way track members by the open-arc process.

45 Another object is to provide an improved tube rod or coil that will consistently produce deposits of the highest degree of quality and dependability.

Still another object is to provide an improved semi-automatic arc welding process.

Other aims and objectives of this invention will become apparent from the present disclosure.

These and other objects are obtained through the provision of a novel hard-facing tube rod consisting of a mild steel sheath and a filler material that is powder-blended, preferably according to Fischer Patent No. 2,514,126, dated July 4, 1950. Such material comprises in weight-percent, about 23 percent chromium, 3 percent combined carbon, and 2 percent free carbon, the particle size of which approaches the molecular, 0.80 percent silicon, 2.75 percent manganese, 2 percent molybdenum, .70 percent aluminum, 1 percent titanium, and the balance iron and incidental impurities together with less than 1 percent of an active fluxing agent. The ratio of sheath to filler material should be about 70 to 30 by weight. The fused deposit of the tube rod consists of 4 to 7 percent chromium, .5 to 1.2 percent carbon, .5 to 1.25 percent manganese, .4 to 1.2 percent molybdenum, .5 percent maximum silicon, up to .1 percent aluminum, up to .25 percent titanium, and the balance iron and incidental impurities, with traces if any, of the fluxing agent. Proper blending of the filler materials is an important and critical feature of the present invention.

In the drawing:

FIG. 1 is a wiring diagram illustrating suitable means for carrying out the invention;

FIG. 2 is an enlarged cross-sectional view of the tube rod, and

FIG. 3 is a fragmentary plan view of a rail joint.

As shown in FIG. 1, when the end of tube-rod electrode 10 is brought into contact with the top of rail 12 to be repaired, a welding circuit is established which includes D.C. source 14, conductor 16, relay coil 18, feed rolls 20, tube-rod electrode 10, rail 12, and ground lead 22. This energizes welding arc 24, and at the same time, closes relay contacts 26, energizing rod-feed motor 28 from generator 30, which drives rod-feed rolls 20 feeding tube-rod electrode 10 from a rod 32 toward the arc 24 as long as the end of such electrode is held near the rail 12.

The operator merely moves guide tube 34 through handle 36 to apply weld metal 38, FIG. 3 on the battered and depressed area of the rail end as may be required to complete the necessary build-up.

As shown in FIG. 2, the tube-rod electrode 10 consists of a steel sheath 40 containing the filler material 42 of the invention.

To obtain desired proportion of elements in the filler material, ingredients in the form of -30 screen size powder, as shown in Table 2, are blended thoroughly, and incorporated within a mild steel sheath. A suitable sheath material is the common SAE 1010 steel.

Chromium is present in the iron-base alloy deposit as a carbide former to provide strength and hardness. Manganese and molybdenum are present in the deposit to

provide impact strength, wear resistance, and hardness. Although chromium, manganese and molybdenum may each vary in content, as shown in Table 2, it is preferred that their total content in the deposit should be not less than about 6 percent. Silicon may be present as an impurity up to about 0.5 percent. Aluminum and titanium may be present as residual elements up to about .1 and .25 percent, respectively, in the deposit; however, these elements are usually lost during the hard-facing operation. The aluminum-titanium compound in the filler serves as a deoxidizing and fluxing agent. Potassium titanate is present in the filler also as a fluxing agent. Carbon is essential in the deposit alloy principally as a carbide former to provide hardness, wear resistance, and strength. The balance of the deposit alloy is iron and the usual impurities associated with this class of alloys; i.e. phosphorus, sulphur and the like. These impurities should be kept at a very low content, consistent with the requirements of railroad mainline specifications.

The filled tube rods may be flash coated with copper to improve electrical contact, inhibit rust and to act as a lubricant for feeding mechanism. Preferably, the mild steel strip is copper coated before it is fashioned as the tube sheath.

TABLE 2  
Composition of filler material

|    | Amount Added, Percent by Weight | Material                                                                                                                                                                                                                                                                                                                                                                                                                                                                                   | Approximate Particle Size |
|----|---------------------------------|--------------------------------------------------------------------------------------------------------------------------------------------------------------------------------------------------------------------------------------------------------------------------------------------------------------------------------------------------------------------------------------------------------------------------------------------------------------------------------------------|---------------------------|
| 30 | 36.00                           | High-Carbon Ferrochrome<br>Carbon, 7.00 percent maximum.<br>Chromium, 66.00 to 69.00 percent<br>Silicon, 1.00 to 3.00 percent.                                                                                                                                                                                                                                                                                                                                                             | -30 mesh.                 |
| 35 | 3.30                            | Standard Ferromanganese (Low Phosphorus Grade).<br>Manganese, 78.00 to 80 percent.<br>Carbon, 7.00 percent maximum.<br>Silicon, 2.00 percent maximum.<br>Phosphorus, .10 percent maximum.                                                                                                                                                                                                                                                                                                  | -30 mesh.                 |
| 40 | 4.50                            | Ferromolybdenum.<br>Molybdenum, 62.00 to 64.00 percent.<br>Silicon, 0.20 to 0.60 percent.<br>Carbon, 0.018 to 0.064 percent.<br>Copper, 0.13 to 0.21 percent.<br>Sulphur, 0.02 to 0.10 percent.<br>Phosphorus, .01 to 0.023 percent.                                                                                                                                                                                                                                                       | -30 mesh.                 |
| 45 | 52.95                           | Iron Powder (Loss in hydrogen 2.00 percent maximum).<br>Metallic Iron, 97.00 percent maximum.<br>Carbon, 0.08 percent maximum.<br>Manganese, 0.20 percent maximum.<br>Sulphur, 0.025 percent maximum.<br>Phosphorus, 0.02 percent maximum.<br>Silica, 0.15 percent maximum.<br>Aluminum-Titanium (High Purity).<br>Aluminum, 45.00 to 46.00 percent.<br>Titanium, 53.00 to 54.00 percent.<br>Iron, 0.50 to 1.00 percent.<br>Silicon, 0.01 to 0.09 percent.<br>Carbon, Nil to 0.08 percent. | -100 mesh.                |
| 50 | 1.00                            | Lamp Black.                                                                                                                                                                                                                                                                                                                                                                                                                                                                                | -100 mesh.                |
| 55 | 2.00                            | Potassium Titanate.                                                                                                                                                                                                                                                                                                                                                                                                                                                                        | -325 mesh.                |
|    | 0.25                            |                                                                                                                                                                                                                                                                                                                                                                                                                                                                                            | -200 mesh.                |

TABLE 3  
Range of Compositions, in w/o

|               | Filler Material |       |         | Rail Deposit |         |         |
|---------------|-----------------|-------|---------|--------------|---------|---------|
|               | Preferred       | Broad | Optimum | Preferred    | Broad   | Optimum |
| Cr            | 20-25           | 18-30 | 23      | 5-7.5        | (4-9)   | 6.5     |
| C (combined)  | 2-4             | 1-5   | 3       | .6-1.2       | .5-1.5  | .9      |
| C (free)      | 1-3             | .5-3  | 2       | Nil          | Nil     | Nil     |
| Mn            | 2-3.25          | 1.5-4 | 2.75    | .5-1.5       | 3-2.5   | 1.0     |
| Mo            | 1-3             | .5-4  | 2.0     | .5-1.5       | 3-2.5   | 1.0     |
| Al            | .5-1            | 2-1.5 | .7      | .2 max       | .2 max  | .1 max  |
| Ti            | .5-1.2          | 2-1.5 | 1.0     | .2 max       | .25 max | .15 max |
| Si            | .5-1            | 2-1.5 | .8      | .5 max       | .5 max  | .3 max  |
| Fe (combined) | Bal             | Bal   | Bal     | Bal          | Bal     | Bal     |
| Fe (free)     | 40-60           | 30-60 | 50      | Nil          | Nil     | Nil     |

Best results are obtained when two percent by weight of amorphous carbon is blended into the filler powder as free carbon. Free carbon in the filler mixture stabilizes the arc, thereby promoting a steady "burn-off" rate. By an undetermined mechanism, the amorphous carbon tends to stabilize the arc. The stabilized arc provides a more uniform control of the fusion of the weld deposit, and especially the depth of penetration at a lower amperage. (Heretofore, high amperages had to be used to make up losses due to unstable arc performance.)

The "burn-off" rate refers to the rate of consumption of the tube-rod during the depositing operation. The stabilized arc promotes a uniform rate of deposition, and therefore, the process is less complicated and may be performed by semi- or even unskilled operators. Further, the uniformly high quality of the deposit renders it suitable for railroad right-of-way maintenance.

Lampblack is especially effective as the amorphous carbon addition, especially when blended, so that its form approaches molecular size, with the other powdered ingredients of the filler. The exact mechanism underlying criticality of lampblack in the composition is not clearly understood. It is tentatively proposed that the amorphous carbon, when added in the form of lampblack, is combined with oxygen in the heat of the arc, thereby providing a  $\text{CO}_2$  envelope to protect the deposit puddle. Other forms of carbon that are crystalline, such as graphite, carbon dust, carbon ash products, and the like, do *not* readily provide the  $\text{CO}_2$  envelope.

Equivalents of lampblack may be deposit products of the flame resulting from the incomplete combustion of carbonaceous materials or gases. These may include flame deposits of acetylene, natural or producers gas, petroleum products and the like. It is believed that the amorphous structure of such soot deposits combines more readily with oxygen to form the  $\text{CO}_2$  envelope. Further, the amorphous carbon is consumed during the hard-facing operation, and does not deleteriously affect the carbon content of the deposited alloy. Experiments show that, when crystalline carbon alone is used as the free carbon in the tube rod in open-arc operations, the carbon behaves erratically in the puddle and yields an alloy with an unpredictable carbon content. Since the presence of amorphous carbon provides an oxygen-deficient atmosphere, when carbon additions to the deposit are desired, crystalline carbon may be added to the tube-rod filler powder along with the amorphous carbon, in sufficient quantities to obtain a predictable carbon content in the deposit. This constitutes a further improvement in the art.

Moreover, it is believed that the amorphous carbon is not readily wetted by the molten metal and, therefore, is less likely to be incorporated into the composition of the deposit alloy. The amorphous carbon will tend to float on the puddle because of its lower specific gravity. A comparison of the properties of the two forms of carbon is given in Table 4.

TABLE 4  
Physical and chemical properties of carbon

| Property                                                                         | Amorphous Carbon | Crystalline Carbon or Graphite |
|----------------------------------------------------------------------------------|------------------|--------------------------------|
| Structure.....                                                                   | Amorphous.....   | Hexagonal-Crystalline.         |
| Molecular weight.....                                                            | 12.01.....       | 12.01.....                     |
| Specific gravity.....                                                            | 1.87.....        | 2.25.....                      |
| Sublimation Temperature, $^{\circ}\text{C}$ .....                                | 3,652-3,697..... | 3,652-3,697.....               |
| Boiling Point, $^{\circ}\text{C}$ .....                                          | 4,200.....       | 4,200.....                     |
| Heat of Combustion, Kg.-Cal./gr-atom.....                                        | 8.08.....        | 7.9.....                       |
| Heat of Oxidation, Cals./gram-atom.....                                          | 97.85.....       | 94.81.....                     |
| Thermal Conductivity:<br>B.t.u./hrs. sq. ft./ $^{\circ}\text{F}/\text{ft}$ ..... | 3.....           | 60.....                        |
| CGS units.....                                                                   | .0004.....       | .0117.....                     |
| Soluble in liquid iron.....                                                      | Unknown.....     | Yes.....                       |

The greatest difference in physical properties between amorphous and crystalline carbon appears to be in thermal conductivity. This is probably due to the extremely

porous nature of the amorphous carbon. In theory, it is expected that the amorphous carbon, being more porous and, therefore having a greater surface area, combines with oxygen in the ambient atmosphere more readily than does the crystalline carbon, which is more dense. In addition, the particles of amorphous carbon are inherently very minute when compared to crystalline carbon, which must be mechanically crushed and pulverized into small particles.

EXAMPLE I  
A mixture of filler material for a hard-facing tube rod was prepared in accordance with the preferred composition as shown in Table 2. After blending the mixture for about one hour in a twin-shell type of blender, the material was processed into a  $\frac{7}{16}$ -inch diameter rod. The proportion by weight of the S.A.E. 1010 steel sheath to filler material was 70 to 30. The method of preparing various sizes of tube-rod (for example,  $\frac{1}{16}$ - to  $\frac{5}{16}$ -inch diameter), while maintaining an established sheath-to-filler ratio is well known in the art.

The tube rod was prepared in the form of a coil with a "flash" coating of copper for the reasons mentioned above. Methods of flash plating the mild steel sheath material are well known in the art. The copper plating is very thin (less than 1 mil) and is probably vaporized and/or oxidized in the heat of the arc. The residual copper content, if any, is only in trace quantities and does not adversely affect the deposit quality.

The tube-rod was "open-arc" deposited on a plate of SAE 1020 steel with a welding current of 275 amperes and 30 volts (direct current-reverse polarity). To obtain a smooth deposit, the weld beads were overlapped approximately 25 percent. Three layers were deposited; the entire deposit was then cold-work hardened by peening. Hardness values for each layer and the work-hardened deposit are shown in Table 5.

Duplicate compositions were prepared to check the reproducibility of the tube-rod. The compositions are identified as Heat No. 7 and Heat No. 36. Each heat was prepared into a number of coils. Hardness values of deposits from random coils are shown in Table 5.

TABLE 5  
Composition and hardness of selected heats

| 45 | Heat No. 7 Composition, weight percent |         | Heat No. 36 Composition, weight percent |         |
|----|----------------------------------------|---------|-----------------------------------------|---------|
|    | Filler Powder                          | Deposit | Filler Powder                           | Deposit |
| 50 | Cr.....                                | 23.66   | 6.34                                    | 21.33   |
|    | C.....                                 | 4.83    | .79                                     | 4.55    |
|    | Si.....                                | .82     | .22                                     | .77     |
|    | Mn.....                                | 2.84    | .96                                     | 2.48    |
|    | Mo.....                                | 3.07    | .90                                     | 1.44    |
|    | Al.....                                | .62     | .04                                     | .06     |
| 55 | Ti.....                                | .94     | .02                                     | .14     |

  

| 60               | Hardness, Re |         | Hardness, Re |         |
|------------------|--------------|---------|--------------|---------|
|                  | Range        | Average | Range        | Average |
| Layer No.:       |              |         |              |         |
| 1.....           | 46-49        | 48.5    | 46-51        | 48.8    |
| 2.....           | 39-46        | 42.9    | 42-45        | 43.4    |
| 3.....           | 35-41        | 38.5    | 33-41        | 37.0    |
| Work Hardened:   |              |         |              |         |
| 3.....           | 44-50        | 47.5    | 46-50        | 47.8    |
| 65               | Coil No.:    |         |              |         |
| 1.....           | 53-57        | 55      | 47-49        | 48      |
| 2.....           | 51-54        | 52.5    | 56-60        | 58.8    |
| 3.....           | 52-55        | 53.0    | 57-60        | 58.6    |
| 4.....           | 51-55        | 53.0    | 57-60        | 58.2    |
| 5.....           | 59-61        | 60.0    | 51-54        | 52.5    |
| 6.....           | 57-59        | 58.0    | 50-53        | 51.5    |
| 7.....           | 59-63        | 61.5    | 55-57        | 56.0    |
| 8.....           | 51-54        | 53.0    | 50-53        | 51.5    |
| 9.....           | 54-55        | 54.5    | 50-53        | 51.5    |
| 10.....          | 57-60        | 58.5    | 55-57        | 56.0    |
| 11.....          | 59-60        | 59.5    | 54-56        | 55.0    |
| Total Range..... | 51-63        |         | 47-60        |         |
| Average.....     |              | 56.2    |              | 54.3    |

7  
EXAMPLE 2

While the hardness of a deposit is only a good indication of wear properties, the ideal evaluation of rail characteristics is possible only in actual service of mainline track over a prolonged period of time. Since such testing would be impractical (and even hazardous), the American Association of Railroads (AAR) has erected a rolling load testing apparatus specifically designed for testing various characteristics of rails. In a testing program conducted by AAR personnel, the deposits of the tube-rod of this invention (as described in Table 2) and three typical commercial (known) welding electrodes were subjected to the rolling load test as mentioned above. All test deposits were made on random worn rails by AAR personnel according to standard railroad practices. Data obtained from the tests are given in Table 7. The data show that the deposit of the tube-rod of this invention, Alloy A, was superior to the alloy deposits of commercially known electrodes for railroad service. The tests are normally terminated at 5,000,000 cycles, which is considered to be optimum endurance, or when excessive wear or an anomaly is noted. It is particularly significant that the wear rate of Alloy A was appreciably lower than wear rates of the others.

The favorable results of the rolling load tests on Alloy A warranted advanced testing. Several miles of mainline track of an eastern railroad was designated as a testing site where Alloy A was deposited on worn rail ends by the open-arc process. The deposits are continually inspected and evaluated to determine the wear and endurance characteristics under actual conditions of use in mainline track.

The results of testing the tube-rod in this Example indicate that the tube rod of this invention is highly suitable for rail end hard-facing with a high degree of dependability and reproducibility as required by the railroad specifications.

TABLE 6  
AAR rolling load test results

| Alloy | Test No. | Hardness, BHN |             |            | Completed Cycles | Deposit Wear, Mils | Approximate Wear Rates, mils per $10^6$ cycles |  |  |  |
|-------|----------|---------------|-------------|------------|------------------|--------------------|------------------------------------------------|--|--|--|
|       |          | Rail          | Deposit     |            |                  |                    |                                                |  |  |  |
|       |          |               | Before Test | After Test |                  |                    |                                                |  |  |  |
| A     | A-1      | 262           | 600         | 627-653    | 5,000,000        | 5                  | 1                                              |  |  |  |
|       | A-2      | 277           | 555-600     | 653-665    | 5,000,000        | 25                 | 5                                              |  |  |  |
|       | A-3      | 245           | 578-600     | 653        | 4,000,000        | 15                 | 3.8                                            |  |  |  |
|       | A-4      | 255           | 512-555     | 622-633    | 5,000,000        | 10                 | 2                                              |  |  |  |
|       | A-5      | 262           | 600         | 653        | 5,000,000        | 15                 | 3                                              |  |  |  |
| B     | B-1      | 309           | 311-347     | 324-354    | 990,700          | 39                 | 39                                             |  |  |  |
|       | B-2      | 266           | 306-329     | 332-364    | 2,000,000        | 49                 | 24.5                                           |  |  |  |
| C     | C-1      | 255           | 248-269     | 290-298    | 1,098,100        | 45                 | 44                                             |  |  |  |
|       | C-2      | 273           | 273-277     | 286-311    | 5,040,000        | 47                 | 9.5                                            |  |  |  |
|       | C-3      | 262           | 255-297     | 286-311    | 2,721,000        | 33                 | 13.0                                           |  |  |  |
|       | C-4      | 241           | 260-302     | 321-323    | 1,000,000        | 47                 | 47                                             |  |  |  |
|       | C-5      | 241           | 255-302     | 321-340    | 971,800          | 48                 | 48                                             |  |  |  |
| D     | D-1      | 286           | 298-307     | 311-356    | 2,000,000        | 55                 | 27.5                                           |  |  |  |

The examples and use of the tube rod of this invention as described herein constitute a preferred embodiment of the invention to provide a clear understanding of the invention, and are not to be construed as limitations except as defined in the appended claims. The tube rods of this invention may be used to provide weldments for hard-facing or joining metal parts other than railway hardware. Weldment deposition may be accomplished by other known work-in-circuit electric arc processes, although the open-arc process is preferred. Other uses and modifications within the scope and spirit of this invention will suggest themselves to persons skilled in the art.

8  
What is claimed is:

1. An arc welding tube rod filler material composed of a -30 screen size powder-blend of the following ingredients, by weight:

|    |               |         |
|----|---------------|---------|
| 5  | Cr            | Percent |
|    | C (combined)  | 1-5     |
|    | C (free)      | 0.5-3   |
|    | Mn            | 1.5-4   |
|    | Mo            | 0.5-4   |
|    | Al            | 0.2-1.5 |
|    | Ti            | 0.2-1.5 |
|    | Si            | 0.2-1.5 |
|    | Fe (combined) | Bal.    |
| 15 | Fe (free)     | 30-60   |

wherein such free carbon is in an amorphous state, such as lampblack, of almost molecular particle size.

2. An arc welding tube rod filler material composed of a -30 screen size powder-blend of the following ingredients, by weight:

|    |               |         |
|----|---------------|---------|
| 20 | Cr            | Percent |
|    | C (combined)  | 2-4     |
| 25 | C (free)      | 1-3     |
|    | Mn            | 2-3.25  |
|    | Mo            | 1-3     |
|    | Al            | 5-1     |
|    | Ti            | .5-1.2  |
| 30 | Si            | .5-1    |
|    | Fe (combined) | Bal.    |
|    | Fe (free)     | 40-60   |

35 wherein such free carbon is in an amorphous state, such as lampblack, of almost molecular particle size.

3. An arc welding tube rod filler material composed

of a -30 screen size powder-blend of the following ingredients, by weight:

|    |               |         |
|----|---------------|---------|
| 65 | Cr            | Percent |
|    | C (combined)  | 3       |
|    | C (free)      | 2       |
|    | Mn            | 2.75    |
| 70 | Mo            | 2.0     |
|    | Al            | .7      |
|    | Ti            | 1.0     |
|    | Si            | .8      |
|    | Fe (combined) | Bal.    |
| 75 | Fe (free)     | 50      |

wherein such free carbon is in an amorphous state, such as lampblack, of almost molecular particle size.

4. An arc welding tube rod consisting of a mild steel sheath containing a core of filler material as defined by claim 2, in which the proportion by weight of the steel sheath to filler material is of the order of 70 to 30.

5. Method of hard facing work composed of steel, which comprises energizing an electric welding arc between the end of tube rod as defined by claim 4, and such work with a source of direct current at reverse polarity in circuit therewith, and feeding said tube rod toward such arc to obtain a smooth fused deposit of alloy from the tube rod that is welded to the work, consisting of a -30 screen size powder-blended mixture, of 4 to 7 percent chromium, .5 to 1.2 percent carbon, about half of which is in an amorphous form having an almost molecular particle size, .5 to 1.25 percent manganese, .4 to 1.2 percent molybdenum, .5 percent maximum silicon, up to .1 percent aluminum, up to .25 percent titanium, and the balance iron and incidental impurities, with traces, if any, of the fluxing agent.

6. A hard-facing tube rod consisting of a mild steel sheath and a -30 screen size powder blend of filler material comprising, in weight-percent, about 23 percent chromium, 3 percent combined carbon and 2 percent free carbon, 0.80 percent silicon, 2.75 percent manganese, 2 percent molybdenum, .70 percent aluminum, 1 percent titanium, and the balance iron and incidental impurities to-

gether with less than 1 percent of an active fluxing agent, in which the ratio of sheath to filler material is about 70 to 30 by weight, and said free carbon in an amorphous state is uniformly powder-blended with the other ingredients of the filler material so that the particles of free carbon in such blend approach molecular particle size.

7. A work-in-circuit welding tube rod filler material containing a -30 screen size powder-blend of chromium, manganese, molybdenum, silicon, and a fluxing agent said powder-blend comprising of, by weight, about 50 percent iron powder and about 2 percent free carbon, wherein such free carbon is in an amorphous state; and incidental unavoidable impurities normally found in articles of this class; said free carbon having a particle size that approaches the molecular.

8. An arc welding electrode consisting of a wire provided with a core composed of the material set forth in claim 7.

#### References Cited in the file of this patent

#### UNITED STATES PATENTS

|              |                 |       |               |
|--------------|-----------------|-------|---------------|
| 1,629,748    | Stoody          | ----- | May 24, 1927  |
| 1,704,978    | Knott           | ----- | Mar. 12, 1929 |
| 25 1,745,267 | Pennington      | ----- | Jan. 28, 1930 |
| 1,942,364    | Rood            | ----- | Jan. 2, 1934  |
| 3,029,165    | Kihlgren et al. | ----- | Apr. 10, 1962 |